

## UNITED STATES PATENT OFFICE

1,972,111

## COLORATION OF TEXTILE MATERIALS

George Rivat, Lyon, France, assignor to Celanese Corporation of America, a corporation of Delaware

No Drawing. Application February 18, 1932,  
Serial No. 593,884. In Great Britain February  
20, 1931

14 Claims. (Cl. 8—5)

This invention relates to the treatment of textile materials, for example filaments, fibres, threads, or fabrics, and in particular textile materials made of or containing cellulose esters or ethers, 5 to obtain fast colorations thereon.

It has been observed that colorations produced with some dyestuffs and especially with anthraquinone derivatives containing free amino or alkyl amino groups lack fastness to the combined 10 agencies of acid and light. In view of the fact that materials are frequently required to withstand acid treatment and may also come into contact with acid combustion products in the atmosphere, this lack of fastness constitutes a certain 15 drawback to the use of the aforesaid anthraquinone derivatives as coloring matters.

U. S. application S. No. 450,308 filed 6th May, 1930, describes improving the fastness of colorations on textile materials with the aid of one or 20 more alkyl, aryl, or aralkyl derivatives of urea, thiourea, or guanidine. I have now found that the fastness of colorations, and particularly of colorations produced with anthraquinone derivatives containing free amino or alkyl amino or 25 arylamino groups, especially 1:4-diaminoanthraquinone derivatives may be improved by means of thiourea itself.

According to the present invention therefore, the fastness of colorations on textile materials is 30 improved by incorporating in the materials thiourea and retaining said thiourea in the materials in any subsequent treatment to which the materials may be subjected. The incorporation of thiourea may be effected prior to, at the same 35 time as, or subsequent to the coloration of the materials.

The improvement of the fastness of colorations, and particularly colorations produced with the above mentioned anthraquinone derivatives, by 40 means of thiourea may be further accentuated by the simultaneous or separate application to, or incorporation in the materials of inorganic compounds having an alkaline reaction, that is to say, substances which are alkaline and contain an in- 45 organic base, for example an alkali metal or other borate, e. g. borax, or sodium carbonate, disodium hydrogen phosphate, sodium acetate, sodium palmitate, or potassium oleate. The alkaline substance should not be in such concentration, nor 50 should it be so basic or alkaline as to affect deleteriously the material, e. g. by hydrolysis in the case of cellulose ester materials. Other substances adapted to increase the fastness of colorations may also be employed with thiourea in accordance with the present invention, for example 55

the substances mentioned in U. S. Patent No. 1,723,230, U. S. applications S. Nos. 449,082 filed 1st May, 1930, 450,308 filed 6th May, 1930, 523,940 filed 19th March, 1931, 523,941 filed 19th March, 1931, and British application No. 4341/31 filed 11th February, 1931.

The thiourea may be incorporated in the material by any convenient method. Thus for example in the case of artificial filaments of cellulose derivatives the thiourea may be dissolved or otherwise incorporated in the spinning solutions used for the manufacture. For instance, an acetone solution of cellulose acetate containing up to 2 per cent. of thiourea on the weight of cellulose acetate may be spun by dry spinning methods to 70 produce cellulose acetate filaments which are capable of being directly dyed in fast shades with amino anthraquinone dyestuffs. It will be appreciated that care should be taken to avoid any subsequent treatment tending to remove the 75 thiourea from the material.

Preferably however the thiourea is applied either during a process of dyeing the material, or during a finishing treatment or other after-treatment. In these cases the thiourea may be 80 applied in any suitable form. The thiourea may for instance be applied in solution in water, alcohol or other organic solvent. The percentage of thiourea incorporated in the material may vary considerably and excellent results have been obtained by incorporating up to 2 per cent. of thiourea, for example 0.2 to 1 per cent of thiourea, in the material.

The thiourea may be incorporated in more or less concentrated dye preparations yielding by 90 dilution with water, soap solution or the like, dyebaths suitable for the direct coloration of the textile materials in fast shades. The concentrated preparations may be in solid, powdered, paste, or liquid form, and may or may not contain other materials facilitating the application of the thiourea or the dyestuffs. For example they may contain dispersing agents and/or protective colloids to facilitate the dispersion of insoluble dyestuffs or to maintain the dyestuffs in 100 the dispersed state.

The following examples illustrate the invention without being in any way limitative:—

## Example 1

105

A finishing bath is made up containing 6 ccs. per litre of a sulphonated castor oil and sufficient of a concentrated solution of thiourea is then added to it to form a 2% solution of thiourea. A knitted cellulose acetate fabric dyed in blue 110

shades with an alkylated 1:4-diaminoanthraquinone derivative, is impregnated in this bath, centrifuged and dried.

*Example 2*

5 A woven fabric of cellulose acetate is, after dyeing, padded in a bath containing 2 grams per litre of thiourea and 2 grams per litre of borax. The excess liquid is pressed out and the material 10 dried and finished.

15 As already indicated the invention is of particular value in rendering fast to the combined agencies of light and acid coloring matters produced with anthraquinone derivatives containing free amino or alkyl amino or arylamino groups. Coloring matters of this class are capable of yielding valuable colorations on cellulose ester and ether materials which are difficult to secure by means of other coloring matters. For this 20 reason the incorporation of thiourea is most valuable in connection with the treatment of textile materials made of cellulose acetate or other cellulose esters or ethers, for instance cellulose formate, cellulose propionate, cellulose butyrate, or 25 other cellulose ester, or methyl, ethyl, or benzyl cellulose or other cellulose ether, or materials containing such cellulose derivatives associated with other fibres, such for example as wool, cotton, regenerated cellulose and silk. The invention 30 may, however, be applied to the treatment of materials consisting wholly of fibres other than cellulose derivative fibres.

What I claim and desire to secure by Letters Patent is:—

35 1. Method of improving the fastness of colorations on textile materials comprising organic derivatives of cellulose comprising incorporating thiourea in the materials and retaining said thiourea in the materials during any subsequent finishing treatment.

40 2. Method of improving the fastness of colorations on textile materials comprising cellulose acetate comprising incorporating thiourea in the materials and retaining said thiourea in the materials during any subsequent finishing treatment.

45 3. Method of improving the fastness of colorations on textile materials comprising organic derivatives of cellulose dyed with anthraquinone dyestuffs comprising incorporating thiourea in the materials and retaining said thiourea in the materials during any subsequent finishing treatment.

50 4. Method of improving the fastness of colorations on textile materials comprising cellulose acetate dyed with amino anthraquinone dyestuffs

comprising incorporating thiourea in the materials and retaining said thiourea in the materials during any subsequent finishing treatment.

5. Method of improving the fastness of colorations on textile materials comprising incorporating up to 2% of the weight of the materials of thiourea in the materials and retaining said thiourea in the materials during any subsequent finishing treatment.

6. Method of improving the fastness of colorations on textile materials comprising cellulose acetate dyed with amino anthraquinone dyestuffs comprising incorporating up to 2% of the weight of the materials of thiourea in the materials and retaining said thiourea in the materials during any subsequent finishing treatment.

7. Method of improving the fastness of colorations on textile materials comprising incorporating therein thiourea and a substance having an alkaline reaction and retaining said thiourea and the substance having an alkaline reaction in the materials during any subsequent finishing treatment.

8. Method of improving the fastness of colorations on textile materials comprising cellulose acetate dyed with amino anthraquinone dyestuffs comprising incorporating therein thiourea and a substance having an alkaline reaction and retaining said thiourea and the substance having an alkaline reaction in the materials during any subsequent finishing treatment.

9. Method of improving the fastness of colorations on textile materials comprising cellulose acetate dyed with amino anthraquinone dyestuffs comprising incorporating therein thiourea and an alkali metal borate and retaining said thiourea and alkali metal borate in the materials during any subsequent finishing treatment.

10. Colored textile materials comprising organic derivatives of cellulose and containing thiourea.

11. Textile materials comprising organic derivatives of cellulose and colored with an anthraquinone dyestuff and containing thiourea.

12. Textile materials comprising cellulose acetate and colored with an anthraquinone dyestuff and containing thiourea.

13. Colored textile materials comprising organic derivatives of cellulose and containing up to 2% of their weight of thiourea.

14. Textile materials comprising cellulose acetate and colored with an anthraquinone dyestuff and containing up to 2% of their weight of thiourea.

GEORGE RIVAT. 130

60

135

65

140

70

145

75

150